

## UNITED STATES PATENT OFFICE

CAMILLE DREYFUS, OF NEW YORK, N. Y., AND HERBERT PLATT, OF CUMBERLAND, MARYLAND, ASSIGNORS TO CELANESE CORPORATION OF AMERICA, A CORPORATION OF DELAWARE

## FIBER, FABRIC, AND ARTICLE CONTAINING ORGANIC DERIVATIVES OF CELLULOSE

No Drawing. Original application filed September 22, 1925, Serial No. 57,956. Divided and this application filed February 28, 1927. Serial No. 171,722.

This invention relates to new and improved products obtained by weighting yarns, fabrics, textiles, etc., made from or containing organic derivatives of cellulose. This application is a division of U. S. application Serial No. 57,956, filed on September 22nd, 1925.

It is well known that certain woven fabrics made from or containing organic derivatives of cellulose such as cellulose acetate have, (in common with similar fabrics made from other materials), a tendency to "shift" or "slip". Similarly, knitted fabrics, especially circular knit fabrics, made from organic derivatives of cellulose have a tendency to ladder or run. These properties are no doubt due to the smooth surface of the threads constituting the fabric. It is also known that if fabrics made from or containing organic derivatives of cellulose are ironed with a very hot iron, the latter will cause the fabric to melt.

The applicants have now discovered that these objectionable properties of such fabrics, textiles, etc., can be overcome. This they have accomplished by weighting the fabric or textile made from an organic derivative of cellulose with proper weighting agents and under proper conditions. Thus improved properties in a cellulose acetate fabric, for example, can be obtained by treating such a fabric with any suitable weighting agent for such a material, under conditions hereinafter described.

An object of this invention is to provide woven fabrics containing organic derivatives of cellulose whose tendency to "shift" or "slip" is materially lessened or entirely removed. Another object of this invention is to obtain knitted fabrics made of or containing organic derivatives of cellulose which will be completely ladder proof, or one whose capacity to ladder is very greatly lowered. Still another object of this invention is to provide fabrics or articles made of or containing organic derivatives of cellulose whose resistance to heat is appreciably enhanced, which fabrics can, therefore, be ironed at comparatively high temperatures without

melting or otherwise affecting the fabric or article.

The applicants have discovered that the improved fabrics, etc., can be obtained by weighting the same with tannic acid, stannic chloride or any other metallic salt or other agent suitable as a weighting agent. These weighting agents can be applied to the fabric or other material either alone or with the aid of an extraneous swelling agent or agents.

The following examples indicate some of the methods of obtaining the improved products:

## Example I

One (1) part of artificial silk made from cellulose acetate is treated with thirty (30) parts of 40° Tw. solution of stannic chloride ( $SnCl_4$ ) during one-half ( $\frac{1}{2}$ ) hour, at a temperature between 40° and 50° C., then rinsed off in water, then treated with 7° Tw. solution of disodium hydrogen phosphate ( $Na_2HPO_4$ ), and rinsed again, and then treated with 7° Tw. solution of sodium silicate, and washed with or without soap solution. The result will be a substantial increase in weight and volume of the fibers, fabrics and articles.

## Example II

One (1) part of cellulose acetate artificial silk is treated with thirty (30) parts of stannic chloride solution of 40° Tw., at a temperature between 45° and 55° C., during one-half ( $\frac{1}{2}$ ) hour. Then rinse off in water and treat with sodium silicate 7° Tw. and wash with or without soap solution. The result will be a substantial increase in weight and volume of the fibers, fabrics and articles.

## Example III

One (1) part of cellulose acetate artificial silk is treated with thirty (30) parts of 40° Tw. solution of stannic chloride, during one-half ( $\frac{1}{2}$ ) hour, at a temperature between 55° and 65° C., then rinsed off in water and treated with 7° Tw. sodium silicate solution, and washed with or without soap solution. The increase in weight and volume is larger in this case than under Example II.

The above examples are merely illustrative and are not to be considered as limiting the present invention to the specific materials, temperatures, concentrations of solutions etc., set out in the examples, since other materials may also be used for weighting the artificial silk

The products obtained by the above treatments were found to be much improved over 10 the original untreated material. The fabrics had a fuller handle and also possessed improved dyeing qualities.

Other valued and unexpected improvements in the fabrics were also noted. Not 15 only had the weight of the fabrics increased, but the volume of the yarns and fibers comprising the fabric had become materially larger. Thus it was found that a woven fabric which, before being weighted, had a tendency to "shift" or "slip", after being weighted 20 improved considerably in this respect. The tendency to "shift" or "slip" had completely or almost completely disappeared, the extent depending upon the amount of weighting imparted to the fabric. The tendency of the 25 fabric to "shift" or "slip" is lessened as the percentage of weighting absorbed by the fabric is increased.

A similar improvement was noted when 30 knitted fabrics were treated as above. Fabrics which ordinarily have a pronounced tendency or capacity to ladder or run after being weighted had this tendency almost completely removed. This, too, can probably be 35 attributed to the enlargement of the individual fibers or threads constituting the fabric, the enlargement of these threads or fibers causing the contiguous fibers to bind against one another more tightly.

40 Fabrics weighted in accordance with this process were found to have another valuable property—an increased resistance to heat. It is known that fabrics made from cellulose acetate or other organic derivatives of cellulose will melt when ironed with a very hot iron. Such fabrics, however, if weighted are 45 noticeably improved in this respect, as they can be ironed with as hot an iron as can be used safely on any other type of fabric without 50 showing any bad effects as a result.

Thus it will be seen that the products obtained as a result of the applicants' process are not only new but possess valuable properties. These improved properties increase 55 the field of usefulness of materials made from cellulose acetate or other organic derivatives of cellulose, particularly in the textile field. Fabrics, garments, etc., made of or containing cellulose acetate, for example, can now be 60 ironed without necessitating the taking of unusual and troublesome precautions. Also the wearing qualities of the weighted fabrics etc., are superior to those of similar unweighted fabrics.

65 This invention includes within its scope

fabrics, articles, etc., whether the same be made wholly of organic derivatives of cellulose such as, for example, cellulose acetate or whether they be made partially of such organic derivatives of cellulose. Thus, for example, mixed fabrics of cellulose acetate and cotton, cellulose acetate and silk, cellulose acetate and wool etc., which contains a weighting substances such as heretofore outlined are within the scope of this invention. The 70 term organic derivative of cellulose as used in the description and claims is to be construed as including organic esters of cellulose such as cellulose formate, cellulose acetate, cellulose butyrate etc., and cellulose ethers such as 75 ethyl cellulose, methyl cellulose, etc. The term "shifting" in the appended claims is used in its broadest aspect. It is, therefore, to be construed as including "laddering" as 80 well as "slipping" and "shifting".

Having described our invention what we claim and desire to secure by Letters Patent is:

1. A textile material consisting of an organic derivative of cellulose which contains 90 a substance which acts as a weighting and swelling agent, said material having an increased resistance to heat.

2. A textile material comprising an organic derivative of cellulose which contains 95 a substance which acts as a weighting and swelling agent, said material having an increased resistance to heat and its tendency to "shift" reduced.

3. A textile material comprising an organic derivative of cellulose which contains 100 a compound of a metal in insoluble form in such amount that its resistance to heat is increased, the metal compound introduced acting both as swelling agent and weighting 105 agent.

4. A textile material comprising an organic derivative of cellulose which contains a compound of a metal in insoluble form in such an amount that its resistance to heat is 110 increased and its tendency to "shift" is reduced, the metal compound introduced acting both as swelling agent and weighting agent.

5. A textile material consisting of cellulose acetate which contains a substance which acts as a weighting and swelling agent, said material having an increased resistance to heat. 115

6. A textile material comprising cellulose acetate which contains a substance which acts as a weighting and swelling agent, said material having an increased resistance to heat and its tendency to "shift" reduced.

7. A fabric comprising an organic ester 120 of cellulose which contains an insoluble form of tin in such amount that its resistance to heat is increased, the tin compound being the only weighting ingredient present.

8. A fabric comprising an organic ester of 130

cellulose which contains an insoluble compound of tin in such amount that its resistance to heat is increased, and its tendency to "shift" overcome, the tin compound being the only weighting ingredient present.

9. A fabric comprising cellulose acetate which contains an insoluble form of tin in such amount that its resistance to heat is increased, the tin compound being the only weighting ingredient present.

10. A fabric comprising cellulose acetate which contains stannic oxide in such an amount that the resistance of the fabric to heat is increased, the stannic oxide being the sole weighting material present.

11. A fabric comprising cellulose acetate which contains stannic oxide in such an amount that the resistance of the fabric to heat is increased, and its tendency to "shift" overcome, the stannic oxide being the sole weighting material present.

In testimony whereof, they have hereunto subscribed their names.

CAMILLE DREYFUS.  
HERBERT PLATT.

25

30

35

40

45

50

55

60